

## UNITED STATES PATENT OFFICE

2,541,884

N-SUBSTITUTED ISOALLOXAZINES AS  
CATALYSTS IN THE DYE BLEACH  
BATHS FOR COLOR PHOTOGRAPHYFritz W. H. Mueller, Binghamton, N. Y., assignor  
to General Aniline & Film Corporation, New  
York, N. Y., a corporation of DelawareNo Drawing. Application December 30, 1947,  
Serial No. 794,822

12 Claims. (Cl. 95—88)

1

This invention relates to a method of processing photographic color pictures, and particularly to N-substituted isoalloxazines as accelerators for dye bleach baths used in producing dyestuff images from dyed silver images.

It is known that in the production of photographic dyestuff images from diffusely dyed photographic emulsions containing a silver image, the latter image must be treated with a bleach bath which decolorizes or bleaches the dyestuff present in the photographic layer in the areas where the metallic silver is present. The dyes, which are employed in the diffuse dyeing of the silver-halide emulsion layer, are primarily azo dyes of the substantive and acid type, although some basic vat dyes and alizarines may also be employed. The bleaching or decolorization of the dyestuff is accomplished in a bleach bath in which there occurs a simultaneous decolorization of the dye with an oxidation of the metal image at the points where silver is present, i. e., the metallic silver is converted into a silver compound which may be removed subsequently by fixation in a solution of hypo.

The bleach baths, employed in this process, consist of an aqueous solution of a mineral acid or a mineral acid containing an alkali halide, such as potassium iodide, ammonium chloride, or both. Such baths require a relatively long treating time so as to destroy the dyestuff present in situ with the silver image. Long treatment in bleaching solutions of high acidity has the tendency to soften the gelatin of the photographic emulsion containing a silver image and bleachable azo dye. Moreover, by the use of such baths, a lack of definition of the picture usually follows with other undesirable characteristics. In order to avoid these shortcomings, various organic compounds have been proposed as catalysts which, when added to the bleach bath, accelerate the action of said bath and materially reduce the bleaching time.

The most practical catalysts so far suggested are the azines, such as phenazine, 2,3-diaminophenazine, and the like. Although phenazine and its substituted products are effective as accelerators, they are highly colored substances and are substantive to gelatin, i. e., leave a stain in the gelatin layer which is difficult to remove, and, which seriously affects the quality of the final image.

I have discovered that N-substituted isoalloxazines (flavins), although colored substances ranging from reddish-orange to yellow in color, are not substantive to gelatin, do not stain the gelatin layer, and do not affect the quality of the final image. The N-substituted isoalloxazines presumably act as very effective hydrogen

2

carriers becoming readily reduced by the action of the bleach solution with concomitant oxidation of the silver image and destruction of the dye in situ therewith.

5 The N-substituted isoalloxazines are characterized by the following formula:

10



15 wherein R represents an aliphatic group, e. g., methyl, ethyl, propyl, butyl, amyl, hexyl, etc., hydroxyalkyl, e. g., hydroxyethyl, hydroxypropyl, hydroxybutyl, etc., dihydroxyalkyl, e. g., dihydroxypropyl, dihydroxybutyl, dihydroxyamyl, etc., polyhydroxyalkyl, e. g., d-ribityl (from d-ribose), 20 1-arabityl (from 1-arabinose), d-lyxityl (from d-lyxose), d-dulcitol (from d-galactose), d-mannityl (from d-mannose), d-sorbityl (from d-glucose), etc., and the phosphoric acid esters and the mono-, di-, and tri-acetic and succinic acid esters thereof, amino-alkyl group, e. g., aminomethyl, aminoethyl, aminopropyl, ethylaminobutyl, diethylaminobutyl, N-heteroamino alkyl, i. e., piperidinobutyl, morpholinopropyl, and the like, aminohydroxyalkyl, e. g., dimethylamino-hydroxypropyl, diethylaminohydroxypropyl, etc., and their hydrochlorides, carboxyalkyl, e. g., carboxymethyl, carboxyethyl, carboxypropyl, carboxybutyl, etc., aryl, e. g., phenyl, naphthyl, etc., aralkyl, e. g., benzyl, phenylethyl, menaphthyl, and the like, and Z represents the atoms necessary to complete an aromatic or heterocyclic ring, e. g., benzene, naphtholene, anthracene, etc., piperidine, pyridine, pyrimidine, quinoline, methylenedioxy, isopropylidenedioxy, and the like. 30 35 40 45

The aromatic and heterocyclic rings may be substituted in the various positions by alkyl, di-alkyl, hydroxyalkyl, and aminoalkyl groups of the same value as represented by R, amino, halogen, e. g. chlorine or bromine, hydroxy, sulfo, carboxy, nitro, and the like.

The following are examples of N-substituted isoalloxazines employed in accordance with the present invention:

50



7,8,10-trimethylisoalloxazine

Ber. 67, p. 1932, 1934.

3

(2)



7,8-dimethyl-10-hydroxyethylisoalloxazine

Helv. Chim. Acta, 17, p. 1516, 1935.

4



7,8-tetramethylene-10-d-arabitylisoalloxazine

10

Ibid.

(3)



7,8-dimethyl-10-dihydroxypropylisoalloxazine

Helv. Chim. Acta, 17, p. 1516, 1935.

20 (8)

Ibid.

(4)



Riboflavin

J. Am. Chem. Soc. 67, 2165.

25

30

35

40 (9)

50

55 Ibid.

60 (10)

65

70

75 Ibid.



7,8-dimethyl-10-d-lyxitylisoalloxazine

Helv. Chim. Acta, 18, p. 522, 1935.

(5)



Araboflavin

Ibid.



8-methyl-10-(d-dulcetyl)isoalloxazine

(6)



7,8-trimethylene-10-d-ribitylisoalloxazine

Ber. 70B, p. 1302, 1937.



8-methyl-10-(d-mannityl)isoalloxazine

- (13) 
- Ibid.
- (14) 
- 7-ethyl-8-methyl-10-d-ribitylisooalloxazine  
Helv. Chim. Acta, 19, p. 1034, 1936.
- (15) 
- Ibid.
- (16) 
- C<sub>21</sub>H<sub>24</sub>O<sub>6</sub>N<sub>4</sub>  
Riboflavin monosuccinate  
J. Biol. Chem. 160, pp. 293-300, 1945.
- (17) 
- C<sub>25</sub>H<sub>28</sub>O<sub>12</sub>N<sub>4</sub>  
Riboflavin disuccinate  
Ibid.
- (18) 
- C<sub>29</sub>H<sub>32</sub>O<sub>15</sub>N<sub>4</sub>  
Riboflavin trisuccinate  
Ibid.
- (19) 
- C<sub>33</sub>H<sub>36</sub>O<sub>18</sub>N<sub>4</sub>  
Riboflavin tetrasuccinate  
Ibid.
- (20) 
- 10-phenylisoalloxazine  
Ber. 68B, p. 1282, 1935.
- (21) 
- 7,8-dimethyl-10-benzylisoalloxazine  
J. A. C. S. 67, p. 2165, 1945.
- (22) 
- CH<sub>2</sub>CH<sub>2</sub>NH<sub>2</sub>·HCl  
10-aminoethylisoalloxazine hydrochloride  
Helv. Chim. Acta, 19, p. 1029, 1936.
- (23) 
- (CH<sub>3</sub>)<sub>2</sub>N(C<sub>2</sub>H<sub>5</sub>)<sub>2</sub>·HCl  
10-(δ-diethylaminobutyl)-isoalloxazine hydrochloride  
J. A. C. S. 68, pp. 883-7, 1946.
- (24) 
- (CH<sub>3</sub>)<sub>2</sub>N(H<sub>2</sub>-H<sub>3</sub>)<sub>2</sub>·H<sub>3</sub>Cl  
10-(γ-piperidinopropyl)-isoalloxazine hydrochloride  
Ibid.
- (25) 
- Phosphoric acid ester of riboflavin  
Ber. 68, p. 383, 1935.

The foregoing N-substituted isoalloxazines are generally prepared by the condensation of an N-substituted o-aminoaniline and alloxan. The N-alkyl isoalloxazines, with an alkyl group in 10-position higher than methyl (see illustration 1), can be prepared by a method analogous to the one described by Tishler et al., J. Amer. Chem. Soc. 67, p. 2165, 1945, by reacting a 2-alkyl substituted o-phenylenediamine with 5,5-dichlorobarbituric acid. Isoalloxazines, with an alkyl group in either 7- and 8-position or both higher than methyl or ethyl, can also be prepared by Tishler et al.'s method by using N-alkyl substituted phenylenediamine derivatives with the proper alkyl substituents in the 4-, 5-positions as starting materials.

The monophosphoric acid esters of the polyhydroxy isoalloxazines (as shown in illustrations 4 to 14) can be prepared by the method outlined in Ber. 68, p. 383, 1935. The corresponding triacetates can be prepared by the method outlined in Ber. 69, p. 1545, 1936.

The compound shown in illustration 29 is prepared by treating 4,5-methylenedioxy-o-phenylenediamine with alloxan and methylating the resulting product with dimethyl sulfate in a manner analogous to the method described in Ber. 67, p. 1942, 1934.

The compound shown in illustration 30 is prepared by treating 4-chloro-5-nitroisopropylidenedioxobenzene with methylamine, the 4-methylamino-5-nitro derivative is catalytically reduced and the reduced compound treated with 5,5-dichlorobarbituric acid.

The process of preparing isoalloxazines, having a polyhydroxyalkyl group in 10-position, is described in United States Patents 2,238,874 and 2,350,376.

All of the foregoing N-substituted isoalloxazines can be reduced to form leuco derivatives which can be re-oxidized with considerable ease, a factor which greatly adds to their value as accelerators in accordance with the present invention. The reduction can be carried out by well-known chemical means, for example, with sodium hydrosulfite (Ber. 66, 319, 1933), with hydrogen in the presence of palladium oxide (ibid. p. 576), or with zinc dust (Ang. Chem. 47, 318, 1934); it can also be effected with the aid of enzymes which are contained in yeast, muscle, liver, heart, brain and kidney tissue (Ber. 66, 1298-1302, 1933).

The N-substituted isoalloxazines may be employed in any mineral acid bleach bath, such as, for example, hydrochloric, hydrobromic, hydroiodic or phosphoric acid, with or without the presence of an alkali halide, such as sodium or potassium bromide, or iodide, sodium chloride, ammonium chloride, and the like. The concentration of the acid to be employed is dependent upon the character of the gelatin constituting the photographic color emulsion layer or layers. Usually, the concentration of the acid ranges up to 2½ N. I prefer, however, to employ a concentration up to 1 N.

Inasmuch as the N-substituted isoalloxazines are water-soluble yellow to orange dyestuffs, which do not stain the gelatin, the amount employed as catalysts is not critical. The higher the amount within practical limits the greater the catalytic activity. An amount as small as 0.005 gram per liter of bleach bath showed an appreciable bleaching action in silver bearing images. For practical purposes, amounts ranging from 0.005 to 2.5 grams per liter of bleach



6,7-dimethyl-10-d-ribitylisoalloxazine

Proc. Soc. Exp. Biol. Med. 55, p. 184, 1944.



6,8-dimethyl-10-d-ribitylisoalloxazine

Ber. 683, p. 172, 1935.



7,9-dimethyl-10-d-ribitylisoalloxazine

Ibid.



9-aza-10-propylflavin

Ber. 71, p. 1243, 1938.



7,8-methylenedioxy-10-methylisoalloxazine



7,8-isopropylidenedioxy-10-methylisoalloxazine

bath may be employed. While any one of the N-substituted isoalloxazines disclosed and contemplated herein may be employed in any mineral acid bleach bath, I prefer, however, to employ the polyhydroxyisoalloxazines shown in Illustrations 4 to 14 and the acid esters thereof shown in Illustrations 15 to 19 because of their general availability and ease of preparation.

The following examples will illustrate the preparation of a multi-layer color film, in which after exposure, the dye images are obtained by the silver dye bleach process, and the bleach baths containing the N-substituted isoalloxazines as accelerators.

#### EXAMPLE I

Three kilograms of a wet gelatino silver-halide emulsion, containing about 10% gelatin, 4-5% of silver-bromoiodide, 10 cc. of a 10% solution of saponin, and 10 grams of diphenyl biguanide hydrochloride were separated into three equal portions of 1 kilogram each and utilized in the preparation of the final red, green, and blue sensitive emulsions.

##### Red sensitive

To the first portion of a red sensitized wet gelatino silver-halide emulsion there were added 5 grams of a bleachable cyan dye, Direct Sky Blue (C. I. #520).

##### Green sensitive

To the second portion of a green sensitized wet gelatino silver-halide emulsion there were added 1.25 grams of a bleachable magenta dye, Fast Acid Magenta B (C. I. #30).

##### Blue sensitive

To the third portion of a blue sensitized wet gelatino silver-halide emulsion there were added an additional 5 grams of diphenyl biguanide hydrochloride as a dye precipitant and 6.8 grams of a bleachable yellow dye, Dianil Yellow 2R (C. I. #650).

##### Coating

The three final silver-halide emulsions, as above prepared, were coated to a dry thickness of approximately 6 microns upon a cellulose acetate film base (or other suitable support such as baryta coated paper) containing an anti-halo coating. The red sensitive silver-halide emulsion was coated first. Over this coating the green sensitive emulsion was coated followed by a coating of approximately 3 microns dry thickness of a yellow filter prepared in accordance with United States Patents 2,036,546; 2,220,187 or 2,390,707. Over the filter layer the blue sensitive emulsion was coated as the outermost layer.

##### Processing

The finished film, prepared in accordance with the foregoing, was exposed and developed for 15 minutes in a black and white developer of the following composition:

|                            |       |     |
|----------------------------|-------|-----|
| Water                      | cc    | 750 |
| Metol                      | grams | 1.5 |
| Sodium sulfite (anhydrous) | do    | 80  |
| Hydroquinone               | do    | 3   |
| Potassium bromide          | do    | 0.5 |
| Water to make              | liter | 1   |

Short stopped for 3 minutes in a bath of the following composition:

|                |       |    |
|----------------|-------|----|
| Sodium acetate | grams | 20 |
| Acetic acid    | cc    | 10 |
| Water to make  | liter | 1  |

Fixed for 3 minutes in a solution of the following composition:

|                                    |       |     |
|------------------------------------|-------|-----|
| Water                              | cc    | 650 |
| Hypo                               | grams | 240 |
| Sodium sulfite (anhydrous)         | do    | 15  |
| Acetic acid (28% aqueous solution) | cc    | 45  |
| Potassium alum                     | grams | 15  |
| Water to make                      | liter | 1   |

The fixed film was then cut into 6 equal strips and the strips treated for 10-15 minutes in dye bleach baths of the following compositions:

I (a)

|                         |       |     |
|-------------------------|-------|-----|
| Hydrochloric acid, conc | cc    | 250 |
| Water to make           | liter | 1   |

No satisfactory bleaching action on the dyes was observed within 15-30 minutes.

##### I (b)

To I (a) 5 cc. of a 0.1% aqueous solution of riboflavin was added. Appreciable bleaching of the dyes in all silver bearing areas took place.

II (a)

|                         |       |     |
|-------------------------|-------|-----|
| Hydrochloric acid, conc | cc    | 100 |
| Potassium iodide        | grams | 100 |
| Water to make           | liter | 1   |

Slight bleaching action was obtained in the cyan, magenta and yellow layers.

##### II (b)

To II (a) 10 cc. of a 0.1% aqueous solution of riboflavin was added. Complete bleaching in the cyan layer and considerably accelerated bleachings were obtained in the magenta and yellow layers with satisfactory color balance.

III (a)

|                         |       |     |
|-------------------------|-------|-----|
| Hydrochloric acid, conc | cc    | 100 |
| Potassium iodide        | grams | 100 |
| Ammonium chloride       | do    | 100 |
| Water to make           | liter | 1   |

Slight action in cyan and appreciable action in magenta and yellow layers.

##### III (b)

To III (a) 10 cc. of a 0.1% aqueous solution of riboflavin was added. Complete bleach in the cyan layer within 10-15 minutes and considerably accelerated bleachings were obtained in the magenta and yellow layers with satisfactory color balance.

#### EXAMPLE II

The bleaching treatment of Example I was repeated on the same fixed color film strips, with the exception that 7,8,10-trimethylisoalloxazine was substituted for riboflavin with similar results.

#### EXAMPLE III

A halogen silver-bearing layer colored with 75 Diamine Pure Blue FF (Schultz Farbslofttabellen

1931, 7th ed., #308) was treated with a bleach solution of the following composition:

Hydrobromic acid ..... cc 250  
Phosphoric acid ester of riboflavin gram 005  
Water to make ..... liter 1

The dye was completely bleached within 10-15 minutes.

While the present invention has been described in considerable detail with reference to certain preferred procedures, materials, and uses, it is understood that the invention is not limited thereto, that numerous variations may be made in the procedures herein described, and that equivalent materials may be substituted. Thus, for example, azo dyes other than those specifically mentioned and utilized in the foregoing examples, may be bleached satisfactorily, provided they are or can be used in the preparation of multi-layer color film in which, after exposure, the dye images are obtained by the silver dye bleach process. Several hundreds of such dyes are known and further reference to them or to their methods of preparation need not be mentioned herein. Accordingly, the scope of the invention is to be defined by the following claims.

I claim:

1. A dye bleach bath for producing a colored image in a photographic emulsion layer containing a bleachable azo dye and a silver image consisting of an aqueous solution of hydrochloric acid, ammonium chloride, potassium iodide and an accelerating amount of an agent selected from the group consisting of N-substituted isoalloxazines corresponding to the following general formula:



where R represents a member selected from the class consisting of aliphatic and aryl groups, and Z represents the atoms necessary to complete a member selected from the class consisting of aromatic and heterocyclic ring systems.

2. A dye bleach bath according to claim 1 in which the accelerating agent is riboflavin.

3. A dye bleach bath according to claim 1 in which the accelerating agent is 7,8,10-trimethylisoalloxazine.

4. A dye bleach bath according to claim 1 in which the accelerating agent is the phosphoric acid ester of riboflavin.

5. The process of producing a colored image in an exposed and developed photographic layer

containing a silver image and a bleachable azo dye which comprises bleaching said layer in a bath comprising an aqueous solution of a mineral acid and an accelerating amount of an agent selected from the group consisting of N-substituted isoalloxazines corresponding to the following general formula:



where R represents a member selected from the class consisting of aliphatic and aryl groups, and Z represents the atoms necessary to complete a member selected from the class consisting of aromatic and heterocyclic ring systems.

6. The process according to claim 5 in which the accelerating agent is riboflavin.

7. The process according to claim 5 in which the accelerating agent is 7,8,10-trimethylisoalloxazine.

8. The process according to claim 5 in which the accelerating agent is the phosphoric acid ester of riboflavin.

9. A dye bleach bath according to claim 1 in which the accelerating agent is araboflavin.

10. A dye bleach bath according to claim 1 in which the accelerating agent is 8-ethyl-10-d-ribitylisoalloxazine.

11. The process according to claim 5 in which the accelerating agent is araboflavin.

12. The process according to claim 5 in which the accelerating agent is 8-ethyl-10-d-ribitylisoalloxazine.

FRITZ W. H. MUELLER.

#### 40 REFERENCES CITED

The following references are of record in the file of this patent:

#### UNITED STATES PATENTS

| Number    | Name   | Date          |
|-----------|--------|---------------|
| 2,221,793 | Gaspar | Nov. 19, 1940 |
| 2,270,118 | Gaspar | Jan. 13, 1942 |
| 2,341,034 | Gaspar | Feb. 8, 1944  |
| 2,410,025 | Gaspar | Oct. 29, 1946 |

#### 45 OTHER REFERENCES

Handbook of Chemistry, Lange, 6th edition, Handbook Publishing Co., Sandusky, Ohio. Sept. 1946; page 738 particularly cited.

Journal of the American Chemical Society, 67; page 2165.

Berichte der deutschen Chemischen Gesellschaft, 67, p. 1932, 1934.